

May 19, 1970

H. L. TAYLOR

3,512,574

CONTINUOUS CASTING PROCESS AND APPARATUS

Filed Dec. 2, 1966

2 Sheets-Sheet 1



Fig. 1

Inventor

Harold L. Taylor

By Hibben, Noyes & Bicknell  
Attorneys

May 19, 1970

H. L. TAYLOR

3,512,574

## CONTINUOUS CASTING PROCESS AND APPARATUS

Filed Dec. 2, 1966

2 Sheets-Sheet 2



Fig. 2

Inventor  
Harold L. Taylor  
By Hibben, Noyes & Bicknell  
Attorneys

3,512,574  
CONTINUOUS CASTING PROCESS AND  
APPARATUSHarold L. Taylor, Hammond, Ind., assignor to Inland  
Steel Company, Chicago, Ill., a corporation of Dela-  
wareFiled Dec. 2, 1966, Ser. No. 598,759  
Int. Cl. B22d 11/12

U.S. Cl. 164—89

5 Claims

## ABSTRACT OF THE DISCLOSURE

A method and apparatus for secondary cooling of a continuous casting as the casting is withdrawn from a continuous casting mold in which the entire surface of the casting is contacted within an enclosure with a narrow stream of cooling medium flowing in turbulent flow which withdraws heat from the casting at a flux density of at least 75 calories per square centimeter per second. The cooling medium for the secondary cooling can be provided by directly connecting the casting mold cooling chamber and the secondary cooling enclosure.

The present invention relates generally to continuous casting of ferrous metals and more particularly to an improved process and apparatus for cooling a ferrous metal continuous casting.

The general principles of producing a continuous casting of a ferrous metal are well known and include the steps of introducing molten metal into an open-ended mold the walls of which are cooled to form an outer shell or skin of solidified metal about a core of molten metal and permitting substantially continuous withdrawal of the casting from the mold. After leaving the mold, the continuous casting usually passes through a secondary cooling zone wherein cooling fluid is applied directly onto the surface of the casting to complete solidification of the molten metal in the interior of the continuous casting.

There have been numerous commercial applications of the continuous casting process for ferrous metals, but there still remain deterrents to greater commercial use, such as the limited rate of production due to the relatively slow rate of withdrawal of the casting from the mold and the occurrence of metallurgical variations and defects in both the surface and internal metallurgical structure of a ferrous metal continuous casting.

While a considerable amount of work has been done on the problem of removing heat from the continuous casting mold, relatively little study has been made of ways and means of removing heat from the incompletely solidified continuous casting after the casting has been withdrawn from the mold. The most common commercial practice in present day continuous casting installations is to spray water onto the surface of the casting to effect the required secondary cooling of the casting, although spraying the cooling fluid is an inefficient means of removing heat and tends to cause metallurgical defects in the casting.

Thus, one of the major problems remaining in the continuous casting of ferrous metals is the effective removal of heat from the incompletely solidified metal casting after it has been withdrawn from the continuous casting mold, since this has a substantial effect on the rate of casting and on the metallurgical structure of the casting.

It is therefore an object of the present invention to provide an improved process and apparatus for more

economically producing ferrous metal continuous castings.

It is a further object of the present invention to provide an improved method and apparatus for removing heat from a continuous casting after withdrawal of the casting from the continuous casting mold.

Other objects of the present invention will be apparent to one skilled in the art from the detailed description and claims to follow when read in conjunction with the accompanying drawing wherein:

FIG. 1 is a schematic vertical sectional diagram of an apparatus for performing the process of the present invention; and

FIG. 2 is a schematic vertical sectional diagram of a modified apparatus for performing the process of the present invention.

It has been discovered that the above specified objects and other objects of the present invention can be achieved by employing a process of cooling a ferrous metal continuous casting in a channel quenching secondary cooling zone to very substantially increase the heat withdrawal flux density and effect more rapid complete solidification of the continuous casting. It has now been found desirable and possible with the channel cooling apparatus of the present invention, for example, to effect a uniform heat withdrawal flux density of at least 75 cal./cm.<sup>2</sup>/sec. (1,000,000 B.t.u./hr./ft.<sup>2</sup>) in the secondary cooling zone.

The channel cooling apparatus and process of the present invention is principally concerned with effecting cooling of a continuous casting after the casting has been withdrawn from the open end casting mold and has as an essential feature thereof contacting the entire lateral surface of the continuous casting as it is withdrawn from the mold with a continuous film or stream of a cooling medium flowing in turbulent flow. One apparatus for effecting the secondary cooling of a continuous casting in accordance with the present invention is shown schematically in FIG. 1 of the drawing, wherein molten ferrous metal is poured into the inlet end of a continuous casting mold 10 of any suitable design. A mold suitable for continuously casting a 200 mm. by 1500 mm. steel slab normally would have a length of about 600 mm. The mold 10 preferably has a plurality of cooling fluid inlets 11 and cooling fluid outlets 12 to allow circulation of cooling fluid through the mold 10 to effect rapid solidification in the mold of an outer shell or skin portion 13 about a fluid inner core of the molten metal 14. A secondary cooling channel quenching apparatus 20 extends downwardly from the lower end wall of the mold 10 and is disposed to receive in the axially extending passage thereof the partially solidified continuous casting as it is withdrawn from the lower end of the mold 10. A plurality of pinch rolls 35 are mounted immediately below the lower end of the secondary cooling apparatus 20 for drawing the casting through the apparatus. The pinch rolls 35 also serve to deflect water away from the casting surface into an exhaust water receiver 36 which surrounds the lower end of the channel quenching apparatus 20 and the pinch rolls 35. A deflector apron 37 with air jets 38 are mounted below each of the pinch rolls 35 and direct the flow of cooling fluid away from the surface of the pinch rolls 35.

The channel quenching secondary cooling apparatus 20 of the present invention comprises a tubular shaped cooling wall 21 having a depth and width larger than the depth and width of the continuous casting and adapted to receive the continuous casting in the axial passage extending therethrough and providing a relatively narrow cooling liquid flow channel 22 about the entire perimeter of the continuous casting for conveying a continuous stream of a cooling fluid between the

inner surface of the cooling wall 21 and the outer surface of the shell 13 of the continuous casting. The width of the flow channel 22 can range between about 0.5 cm. and 5.0 cm., and preferably is about 1.0 cm. The cooling wall 21 can be made of any material, such as cooper or steel, which is sufficiently heat resistant to withstand the relatively high temperatures encountered in the continuous casting of a ferrous metal.

At the upper end of the cooling wall 21 is a chamber 25 which receives a supply of cooling fluid, such as water, and feeds the cooling fluid to the upper or inlet end of the flow channel 22 formed about the continuous casting by the cooling wall 21. The chamber 25 is formed of a lateral wall section 26 and a lower wall section 27 which is welded or otherwise sealably secured to the outer surface of the cooling wall 21 at a point spaced from the upper end thereof and an upper wall section 28 which preferably also serves as the lower wall of the casing mold 10. The upper wall section 28 is spaced above the upper end of the cooling wall 21. A baffle member 29 extends downwardly from the inner surface of the upper wall section 28 and terminates short of the lower wall sections 27. One or more cooling fluid inlets 30 are provided in the lateral wall sections 26 adjacent the upper edge thereof. The chamber 25 is also preferably provided with interior support means 31 which can be ribs, rods or tubes extending supportively between the cooling wall 21, the baffle means 29, and the lateral wall 26 to provide lateral support for the upper end of the wall 21 and to maintain the dimensional spacing of the vertically dispersed members 21, 25 and 29 of the chamber 25. The support means 31 is designed to minimize any restriction of the flow of cooling water and avoid localized heat withdrawal from the wall 21.

In a modified form of the apparatus of FIG. 1, the cooling fluid inlet of the flow channel 22 of quenching apparatus is operatively combined with the cooling liquid outlet of continuous casting mold 10. Thus, as shown in FIG. 2, a continuous casting mold-channel quenching apparatus 40 has a casting mold wall 41 which receives the molten ferrous metal and which shapes the molten metal into the desired form of continuous casting 32. A cooling chamber 42 is formed integrally with the upper end of the mold wall 41 by providing a top wall section 43 connected to the upper end of the mold wall 41, a lateral wall section 44 and a lower wall section 45 which is spaced from the lower end of the mold wall 41. An outer baffle member 46 extends downwardly from the upper wall section 43 intermediate the ends thereof with the lower edge of the outer baffle member 46 being spaced from the lower wall section 45 to provide a fluid passage for cooling fluid introduced by means of one or more fluid inlets 47 in the lateral wall section 44 adjacent the upper edge thereof. The inner edge of the lower wall section 45 is sealably joined with an upwardly extending inner baffle member 48 which projects vertically into the interior of chamber 42 between the baffle member 46 and the casting mold wall 41, terminating short of the upper wall section 43. The inner baffle member 48 is spaced from the mold wall 41 to provide a relatively narrow channel for the flow of cooling fluid over the outer surface of the mold wall 41 to effect rapid heat withdrawal therefrom. The cooling chamber 42 is also preferably provided with interior support means 49 which can be ribs, rods or tubes, extending supportively between the mold wall 41, the inner baffle member 48, the outer baffle member 46, and the lateral wall section 44 to provide lateral support and dimensional stability for the vertically disposed members 41, 44, 46 and 48 of the cooling chamber 42. The support means 49 is designed to minimize any restriction of the flow of cooling water and avoid undue localized heat withdrawal from the mold wall 41.

The lower end of the baffle member 48 is integrally connected, preferably by means of a short tapered section 50, with an elongated cooling channel-defining wall member 51 which extend axially beyond the lower end of the mold wall 41 and is adapted to receive in the axial passage thereof the continuous casting as it leaves contact with the mold wall 41. The dimensions of the wall member 51 are such as to form a relatively narrow but substantially uniform cooling or quenching channel 52 between the outer surface of the continuous casting and the inner surface of the wall member 51 for the flow of cooling fluid. The width of the quenching channel 52 is preferably the same as the spacing between the outer surface of the mold channel wall 41 and the baffle member 48. While the uniform channel 52 width can be as narrow as 0.5 cm. or as large as about 5.0 cm., in the preferred form the width of the channel is maintained at about 1.0 centimeter.

A plurality of water reflecting pinch rolls 55 engage the outer surfaces of the continuous casting immediately below the lower end of the wall member 51 to direct the flow of cooling fluid away from the continuous casting 32 into the exhaust water receiver 56. An apron 57 and air jets 58 are mounted below the pinch rolls 55 to remove cooling fluid from the surface of the pinch rolls 55.

In the operation of the secondary cooling channel quenching apparatus 20 of FIG. 1, cooling fluid, such as water, is introduced through the water inlets 30 of the cooling chamber 25 wherein the baffles 29 uniformly distribute the cooling fluid which passes downwardly through the passage defined by the outer wall section 26 and baffle 29 and then upwardly over the upper end wall of the cooling wall 21 into the cooling channel 22 where the cooling water flows directly into contact with the surface of the solidified shell of the continuous casting and passes downwardly in continuous turbulent flow over the entire perimeter of the continuous casting and outwardly past the lower end of the cooling wall 21. The pinch rolls 35 which are in substantially sealing engagement with the surface of the continuous casting 32 deflect the cooling water laterally into the exhaust water receiver 36. The apron 37 and air jets 38 which are directed against the periphery of the pinch rolls 35 assist in deflecting the cooling water into the exhaust water receiver 36 and away from the surface of the continuous casting 32. If desired, the cooling water can be recycled for use in the secondary cooling channel quenching apparatus 20 or for cooling the casting mold 10.

In operating the modified form of apparatus shown in FIG. 2, cooling fluid, such as water, is introduced through fluid inlets 47 into the casting mold cooling chamber 42 wherein the baffle member 46 evenly distributes the inflowing cooling water, directing the flow downwardly through the passage formed between the lateral wall section 44 and baffle 46 and then upwardly over the upper end of the baffle member 48 into contact with the outer surface of the mold wall 41 and downwardly into and through the secondary cooling channel 52. The cooling water then leaves the lower end of the cooling channel 52 and is deflected laterally by the pinch rolls 55 into the exhaust water receiver 56. The apron 57 and air jets 58 assist in deflecting the water from the pinch rolls 55 and casting 32 into the receiver 56.

In the continuous casting of a ferrous metal in accordance with the present invention, a generally rectangular slab of a low carbon steel having a width of 1500 mm. (60 inches) and a thickness of 200 mm. (8 inches) can be cast at a production rate of about 1.42 metric tons per minute (equivalent to a slab withdrawal speed of about 60.4 cm./min. or approximately 24 inches per minute) using a water flow rate of 10.3 m.<sup>3</sup> per minute through the cooling channel formed about the

entire lateral surface of the continuous casting slab with the cooling water having a velocity of 500 cm./sec. (16.4 ft./sec.) through the secondary cooling channel which has a length of 100 cm. (3.28 ft.) and a channel width of 1.0 cm. (.393 inch). A heat withdrawal flux density in excess of 75 cal./cm.<sup>2</sup>/sec. (1,000,000 B.t.u./hr./ft.<sup>2</sup>) is attained with the apparatus shown in FIGS. 1 and 2. The temperature of the cooling water is increased about 14.6° C. as it passes through the secondary channel cooling apparatus of FIG. 1, and a temperature increase of about 19° C. is produced when the cooling water passes through the combined casting mold and secondary cooling apparatus of FIG. 2. When using the apparatus of FIG. 1 it is necessary to provide a second source of cooling water for the mold in addition to the cooling water supplied for the secondary cooling channel quenching apparatus. Thus, in the above described continuous casting operation employing the apparatus of FIG. 1, it is necessary to provide cooling water at a rate of about 8 m.<sup>3</sup>/min. for the mold in addition to the 10.3 m.<sup>3</sup>/min. required by the secondary cooling apparatus. With the apparatus of FIG. 2 only the 10.3 m.<sup>3</sup>/min. of cooling water is required, since the cooling water from the mold is used as the source of cooling water for the secondary cooling apparatus.

It will be evident that the method and apparatus of the present invention, by employing relatively small volumes of cooling water and sufficiently high water velocities, can effect a very rapid and uniform, uninterrupted cooling of a ferrous metal continuous casting, while at the same time reducing the likelihood of encountering operational difficulties, such as remelting of the casting skin after withdrawal from the mold and irregular cooling of the continuous casting due to stoppage of one or more cooling sprays.

It will also be evident that when the velocity of the cooling water in the secondary cooling channel is increased to higher values, such as 2000 cm./sec. or 12,500 cm./sec., substantially higher heat withdrawal flux densities and casting rates can be achieved. For example, when the water velocity in the secondary cooling channel is 2000 cm./sec. through a channel 100 cm. long having a width of 1.0 cm. and a water flow rate of 41.2 m.<sup>3</sup>/min., a heat withdrawal flux density of 150 cal./cm.<sup>2</sup>/sec. ( $2 \times 10^6$  B.t.u./hr./ft.<sup>2</sup>) and a casting rate of approximately 2.84 metric tons per minute can be achieved. At a cooling water velocity of 2000 cm./sec. in the apparatus of FIG. 1, the temperature of the cooling water in the secondary cooling channel is increased about 7.3° C. and in the apparatus of FIG. 2 the water temperature is increased approximately 10° C. With a water velocity of 12,500 cm./sec. in the secondary cooling channel of the present invention, a heat withdrawal flux density of 375 cal./cm.<sup>2</sup>/sec. can be achieved.

The term "ferrous metal" as used in the foregoing specification and in the following claims designates any of the various carbon steels and ferrous alloys which are normally continuously cast. A typical continuous steel casting of the present invention which can be used for producing a fully killed commercial quality steel for plate application has the following analysis: .17-.24% carbon, .30-.60% manganese, .15-.30% silicon, .30% maximum phosphorous, and .035% maximum sulfur.

I claim:

1. In a ferrous metal continuous casting apparatus, a secondary channel cooling means comprising an elongated tubular member with an axial passage extending the length thereof and adapted to receive in spaced relation therewith a continuous casting having a solidified shell with a core of molten metal as said casting is withdrawn from a liquid cooled continuous casting mold, the inner

surfaces of said tubular member forming with said continuous casting an elongated cooling channel which has a width of about 0.5 cm. to 5.0 cm. about the entire perimeter of said casting, and a cooling liquid supply means in fluid-flow communication with the upper end of said tubular member adapted to provide within said channel and in direct contact with the surface of said continuous casting a continuous stream of cooling liquid in turbulent flow effecting by means of said cooling liquid a heat withdrawal flux density from said casting of at least about 75 cal./cm.<sup>2</sup>/second.

2. A continuous casting apparatus as in claim 1, wherein in said cooling liquid for said cooling channel is comprised entirely of said liquid from said continuous casting mold.

3. In a method of continuously casting a molten ferrous metal in a fluid cooled open-ended continuous casting mold wherein molten metal is introduced into one end of said mold and continuously forming therein a casting

20 having a solidified shell with a core of molten metal, continuously withdrawing said solidified shell from the opposite end of said mold and further cooling said casting in a secondary cooling zone to complete solidification of said molten metal, the improvement comprising; 25 passing said casting as withdrawn from said mold directly into a cooling chamber defining said secondary cooling zone having an elongated cooling medium flow channel between the outer surface of said shell and the inner surface of said cooling chamber with said flow 30 channel having a width of about 0.5 cm. to 5.0 cm., passing liquid cooling medium through said cooling medium flow channel as a confined stream in direct contact with said shell, and maintaining said stream of liquid cooling medium flowing at a velocity which maintains said 35 stream in turbulent flow while in said channel and effecting withdrawal of heat from said continuous casting at a flux density of at least 75 calories per square centimeter per second.

4. A method as in claim 3, wherein said cooling medium flow channel has a width of about 1.0 centimeter.

5. A method as in claim 3, wherein said stream of liquid cooling medium in said secondary cooling zone is provided by direct fluid flow communication between said channel and a cooling chamber of said continuous casting mold, and said cooling medium within said cooling chamber contacting the entire lateral surface of said mold and being maintained in turbulent flow therein.

#### References Cited

##### UNITED STATES PATENTS

|           |         |              |       |           |
|-----------|---------|--------------|-------|-----------|
| 3,324,932 | 6/1967  | Ayers        | ----- | 164-89    |
| 3,354,941 | 11/1967 | Halstead     | ----- | 164-283   |
| 3,358,744 | 12/1967 | Rossi        | ----- | 164-283 X |
| 3,391,725 | 7/1968  | Rossi        | ----- | 164-283 X |
| 3,399,716 | 9/1968  | Rossi et al. | ----- | 164-128 X |
| 894,410   | 7/1908  | Trott        | ----- | 164-283 X |

##### FOREIGN PATENTS

|    |           |         |              |
|----|-----------|---------|--------------|
| 60 | 144,447   | 12/1951 | Australia.   |
|    | 595,254   | 3/1960  | Canada.      |
|    | 1,280,293 | 11/1961 | France.      |
|    | 746,027   | 12/1944 | Germany.     |
|    | 173,322   | 11/1960 | Sweden.      |
| 65 | 233,610   | 11/1944 | Switzerland. |

J. SPENCER OVERHOLSER, Primary Examiner

R. S. ANNEAR, Assistant Examiner

70 U.S. Cl. X.R.

164-283